

## UNITED STATES PATENT OFFICE

2,092,010

SAPONIFICATION OF ORGANIC ESTERS OF  
CELLULOSE

Robert Wighton Moncrieff and Frank Brentnall  
Hill, Spondon, near Derby, England, assignors  
to Celanese Corporation of America, a corpora-  
tion of Delaware

No Drawing. Application May 31, 1935, Serial No.  
24,366. In Great Britain June 16, 1934

11 Claims. (Cl. 8—20)

This invention relates to improvements in the saponification of organic esters of cellulose, and in particular to the saponification of filaments, threads, fibres, ribbons, films and like materials comprising such esters.

U. S. application S. No. 709,335 filed 1st February, 1934, describes the saponification of materials comprising cellulose acetate or other saponifiable ester of cellulose by means of liquid media containing organic bases, and particularly bases such as methylamine. The specification indicates the advantages obtainable by the use of such bases over the use of mineral saponifying agents. Among the most important of these advantages are the enhanced extensibility coupled with high strength of the products and the relatively small loss of weight involved in effecting such a degree of saponification as substantially to change the solubility properties and dyeing properties of the materials, for example to produce from ordinary cellulose acetate materials, materials which have an affinity for cotton dyes, which are insoluble in acetone and which have an enhanced extensibility. Methylamine is particularly advantageous from this point of view.

U. S. application S. No. 752,376 filed 9th November, 1934, contemplates the saponification of materials of the type referred to above by means of liquid saponifying agents containing bases such as ethylene diamine, which have also been found particularly suitable where high tenacity coupled with relatively high extensibility and small loss of weight on saponification are desired.

U. S. applications S. Nos. 756,285 and 756,284 filed on 6th December, 1934, disclose the remarkable acceleration in saponification by means of methylamine, ethylene diamine and like acting organic bases which can be obtained by applying these bases in the presence of even relatively small amounts of metals which are capable of forming amines or like complex nitrogen-containing compounds, and particularly in the presence of copper.

U. S. application S. No. 756,282 filed on 6th December, 1934, describes a process for the saponification of cellulose ester materials by means of methylamine and like bases, wherein saponification is accelerated by the presence of small quantities of strong mineral alkalies or bases, for example caustic soda.

According to the present invention, in the saponification of organic esters of cellulose, a part of the saponification is effected by treatment with an organic base, and the desired saponifica-

tion is completed by a subsequent treatment with a mineral saponifying agent.

Preferably the greater part of the saponification desired should be effected by means of the organic base. Thus it is of advantage in treating materials containing two or more acidyl groups per  $C_6H_{10}O_5$  unit so as to produce complete saponification or at least to saponify to a considerable extent, for example until affinity for cellulose ester dyes is lost, to carry saponification by means of the organic base to the stage where only 1 to  $1\frac{1}{2}$  acidyl groups per  $C_6H_{10}O_5$  unit remain. The product so obtained is then treated with the mineral saponifying agent to complete the saponification desired.

The process of the invention enables results similar to those obtained by the use of methylamine or like acting organic base alone to be obtained much more rapidly than when the whole of the desired saponification is effected by means of such base alone. By the process of the invention filaments, threads, fibres, ribbons, films and like materials may be obtained having an affinity for cotton dyes, a high safe ironing point, high tenacity and good extensibility and elasticity. The process enables substantially complete saponification to be effected in a relatively short time.

The process of the invention is of particular importance in connection with the treatment of filaments, threads, fibres, ribbons, films and like materials of cellulose acetate, and is described herein with particular reference to the treatment of such materials. The process is, however, applicable to the treatment of organic esters of cellulose, i. e. esters of cellulose containing organic acidyl groups, broadly. Among such esters other than cellulose acetate mention may be made of other simple esters of lower fatty acids, for example cellulose formate, propionate and butyrate, esters or higher fatty acid esters, for example cellulose laurate, mixed fatty acid esters, for example cellulose acetate-propionate, cellulose acetate-butyrate and cellulose-acetate propionate-butyrate, ether-esters, for example ethyl cellulose acetate and oxy-ethyl cellulose acetate, and esters containing inorganic radicles, for example nitrocellulose acetate, nitrocellulose acetate-propionate and nitrocellulose acetate-butyrate. The ester content may be that of a completely esterified cellulose. Preferably, however, materials comprising esters of intermediate ester content, for example from 2 to  $2\frac{1}{2}$  ester groups per molecule, are employed. In the case of cellulose acetate, for example, it is preferable to

employ acetates having an acetyl value between 48 and 58%, and preferably between 52 and 54.5% calculated as acetic acid per  $C_6H_{10}O_5$  unit.

The materials treated may be in the form of 5 filaments, threads, yarns, ribbons or the like or of fabrics containing such threads and the like. The organic ester of cellulose employed may be of normal or low viscosity, or of high viscosity, for example in the case of cellulose acetate the 10 viscosity may be of the order of 30 to 50, 100, 200 or even higher, these figures being obtained by comparison of a 6% solution of the ester in acetone at 25° C. with glycerine at the same temperature taken as a standard of 100. Such esters 15 of high viscosity may readily be made by methods in which degradation of the cellulose molecule is substantially avoided during acetylation, for example the methods of U. S. Patent No. 1,708,787. On the other hand, the viscosity of 20 the cellulose acetate employed may be of the order of 10 to 20 or even lower, or between 20 and 30, measured on the scale referred to above.

Any suitable dry or wet spinning method may 25 be employed in producing the filaments and the like. Special mention may be made of the methods described in U. S. applications S. No. 402,785 filed 26th October, 1929, No. 418,414 filed 3rd January, 1930, No. 437,423 filed 20th March, 1930, No. 469,622 filed 21st July, 1930, and No. 30 601,043 filed 24th March, 1932, wherein the materials are produced by wet spinning methods in the course of which they are stretched to a considerable extent. The materials may also, particularly when spun by a dry spinning method, 35 be subjected to a stretching treatment prior to saponification. Such treatments are particularly valuable where a high tensile strength in the products is required, and for this purpose it is of advantage to stretch the materials to a considerable extent, for example to 200, 300 or even more than 500% of their original length. The stretching may be facilitated by any suitable means, e. g. by means of organic swelling agents or as described in U. S. applications S. No. 4,510 40 filed 1st February, 1935 and No. 4,511 filed 1st February, 1935 by means of steam or hot water. The stretching may be effected in a single stage or in several stages, with or without a rest interval between the stages, as described in U. S. 45 application S. No. 573,424 filed 6th November, 1931. If desired after stretching and before saponification the materials may be treated with shrinking agents, as described, for example, in U. S. application S. No. 611,240, filed 13th May, 50 55 1932.

The organic saponifying agent preferably 60 comprises an aqueous solution of methylamine. Other bases of a similar nature may however be employed, among the most important of which 65 is ethylene diamine. The invention moreover includes the use of other strong bases, for example ethylamine, propylamine, amylamine, and triethylamine. Again, somewhat weaker bases of the same series, for example trimethylamine and 70 allylamine, may be used. Further, considerably stronger bases of the same series may be employed, even very strong bases such as tetramethyl ammonium hydroxide, provided care be taken to avoid damaging the materials. The 75 saponifying agent may moreover contain bases of the heterocyclic series, for example piperidine. Again, as described in U. S. application S. No. 752,376, amines other than ethylene diamine containing more than one amino group, and particularly aliphatic diamines of relatively low mo-

lecular weight, for example symmetrical dimethyl ethylene diamine, mono-methyl ethylene diamine, and propylene diamine may also be used. Preferably at least one of the amino groups of such amines should be unsubstituted or mono-substituted. Amines containing more than two amino groups may also be employed, for example 1,2,3-triamino propane. The effect of one or more hydroxy groups in the amine appears to be to favour the penetration of the materials by the saponifying agent, and with this object in view substances of the type of  $\alpha\gamma$ -diamino- $\beta$ -hydroxy propane may be used with advantage. The action of the organic base may be accelerated by the presence of appropriate agents, among which 10 copper and copper salts are of particular importance, as described in U. S. applications S. Nos. 756,285 and 756,284. The presence of small quantities of caustic soda or other mineral alkali may also accelerate the action of the organic 20 base.

The organic saponifying medium is preferably applied to the materials in the form of an aqueous solution. Generally speaking, aqueous concentrations of 15-30% are suitable. Naturally 25 however the most suitable concentration at which a particular base can be employed will depend on the nature of that base. Concentrations below 15%, e. g. 10%, can also be used but in this case saponification is apt to be undesirably 30 slow. The temperatures may range from below atmospheric temperature to the neighbourhood of the boiling point of the solution. Thus the temperature may be between 15 or 20° C. and 35 25 or 30° C. but more rapid saponification occurs at somewhat higher temperatures, e. g. 30-60° C. or more. With a view to preventing excessive evaporation of the organic base saponification 40 may be effected under pressure as described below, or the surface of the saponifying medium 45 may be covered with a layer of oil, wax or other suitable relatively non-volatile substance which is liquid at the temperature of working. Preferably when such substance is used the arrangement is such that the materials treated do not come into contact with the substance. In general, the conditions should be chosen so that the desired degree of saponification may be effected 50 by means of a treatment lasting from 30 seconds or even less up to 1 or 2 minutes. The materials should not be allowed to remain in contact with the saponifying medium after the desired degree of saponification has been effected.

The mineral saponifying agent is preferably 55 applied in aqueous or aqueous-alcoholic solution. Where the mineral saponifying medium contains an alcohol this may itself play a part in the saponification, so that a smaller amount of saponifying agent may be necessary than is theoretically required to give the desired saponification. Among 60 the most useful of mineral saponifying agents is caustic soda. Other alkaline compounds of alkali metals which may be employed are, for example, trisodium phosphate, sodium carbonate, sodium silicate, the corresponding potassium 65 salts and potassium hydroxide. The concentration of the mineral saponifying agent may vary between wide limits. Concentrations of 1 or 2 to 4 or 5% caustic soda or the equivalent of other alkali are very suitable. Considerably lower concentrations may be employed, but in general this involves a more protracted treatment and/or the use of higher temperatures. The temperatures 70 may be of the order of 60 to 70° C., but in some cases, particularly when employing relatively low 75

concentrations of alkali, considerably higher temperatures may be employed with advantage, for example up to 80, 90 or even 100° C.

As indicated above the mineral saponifying solution may contain alcohols. Alcohols may also be contained in the solution of the organic base. These alcohols may or may not have a swelling action upon the cellulose esters treated. Both the mineral saponifying agent and the saponifying agent containing the organic base may if desired contain swelling agents, other than alcohols, for the cellulose esters. For example these solutions may contain acetone, the dimethylene ether of glycol, dioxane, or methylene ethylene ether, all of which substances are swelling agents for cellulose acetate.

The process of the invention is preferably carried out as a continuous operation, the materials being passed, for example, first through a bath containing the methylamine or other organic base and then through a bath containing the mineral saponifying agent. Between the two stages of such a treatment a washing step may if desired be interposed, but this will in general be unnecessary. When the materials are treated in the form of filaments, threads, yarns and the like it is of advantage to effect saponification in warp formation, i. e. by drawing a "warp", i. e. a number of threads in parallel relationship and in the same plane, through baths containing the saponifying agents by means of rollers or like devices extending across the entire warp.

The invention is not, however, limited to carrying out the process in the continuous manner described above. Thus, for example, the materials in hank form may be suspended from rods which are caused to traverse in turn baths containing the organic and the mineral saponifying agents, the rods being caused at the same time to rotate so as to expose each portion of the yarn to the same depth in the bath for the same period. Again, the materials may be treated in the form of bobbins, cheeses or like packages, or in the form of cakes from centrifugal spinning boxes. Any suitable means may in fact be adopted in applying the saponifying agents to the materials. Materials in yarn or like form may be treated continuously with their production and/or with a stretching step. Again, in the case of such materials stretching may be effected during saponification or, provided saponification has not been carried too far, after saponification, as described in U. S. application S. No. 755,232 filed 28th November, 1934. Thus, for example, a stretch may be imparted to the materials while they are in contact with the organic base, particularly if that base has a relatively strong swelling action upon the cellulose ester forming the base of the materials; or stretching may be effected while the materials are in contact with the mineral saponifying agent, provided a swelling agent is present therein.

The materials may be saponified in fabric form. This may conveniently be effected by passing the fabric continuously through a bath containing the saponifying agent, for example in an apparatus of the type of the winch dyeing machine.

It is of advantage to carry out the saponification, and particularly the treatment with the organic base, under pressure. This enables higher temperatures to be employed without undue loss of saponifying agent. The pressure treatment may be applied whether the materials are treated in the form of filaments, threads and the like or of fabrics, and whether the process is

continuous or a batch process. When the process is carried out continuously, the materials may be passed through a closed vessel containing the methylamine or other organic base in solution, under pressure, as described for example in U. S. application S. No. 11,080 filed 14th March, 1935. After leaving the vessel in which saponification with the organic base is effected the materials may pass through a second similar vessel containing the mineral saponifying agent; or this second vessel may be open to the atmosphere. It is of particular advantage to provide the saponification vessel with end pressure chambers, as described in U. S. application S. No. 17,242 filed 19th April, 1935.

The materials prior to saponification may be subjected to a treatment adapted to facilitate penetration of the saponifying agent. This may comprise the application of water to the materials, or they may be treated with aqueous wetting agents, for example soaps.

The degree of saponification effected may be merely sufficient to produce a loss in acidyl content of the order of 10 to 15% or even less, but is preferably somewhat higher, for example sufficient to remove 20 to 30 or 35% of the original acidyl content. Higher degrees of saponification may be effected, sufficient to reduce the acetyl content by 40 to 50 or 60% or more, even up to complete saponification, according to the particular purpose in view. As indicated above it is of advantage when a high degree of saponification is desired to reduce the acidyl content to a single acidyl group per  $C_6H_{10}O_5$  unit by treatment with the organic base and then to complete the desired degree of saponification by means of the mineral saponifying agent.

The following examples illustrate the invention without limiting it in any way:

#### Example 1

Cellulose acetate yarn is passed continuously, in warp formation, first through a bath containing a 15 to 25% aqueous solution of methylamine containing 0.05 to 0.5% copper at 50 to 60° C., and then through a second bath containing a 1 to 3% aqueous solution of caustic soda at a temperature between 90° C. and the boiling point. The yarn emerging from the second bath is washed, dried and collected by suitable means. The speed of travel of the yarn through the baths is adjusted so that by the time the second bath is reached the acetyl content is reduced to an amount corresponding with one acetyl group per  $C_6H_{10}O_5$  unit, and so that the yarn is in contact with the methylamine bath for four or five times as long as with the caustic soda bath.

#### Example 2

The treatment is carried out as in Example 1 except that the treatment with methylamine is carried out under a pressure of 5-10 atmospheres at 80-110° C. the time of treatment being thereby shortened.

In these examples instead of methylamine other organic bases may be employed, e. g. ethylene diamine or ethylamine. The treatment may be carried out as a batch process instead of continuously as described.

What we claim and desire to secure by Letters Patent is:

1. Process for saponifying an organic ester of cellulose, wherein a part of the saponification is effected by treatment with an organic base, and the desired saponification is completed by a sub-

sequent treatment with a mineral saponifying agent.

2. Process for saponifying filaments, threads, fibres, ribbons, films and like materials having a basis of organic ester of cellulose, wherein a part of the saponification is effected by treatment with an aqueous liquid medium which contains a water-soluble nitrogenous organic base in which each carbon atom that is directly attached to a nitrogen atom is directly attached to three other atoms apart from said nitrogen atom, and the desired saponification is completed by a subsequent treatment with a mineral saponifying agent.

15 3. Process for saponifying filaments, threads, fibres, ribbons, films and like materials having a basis of cellulose acetate, wherein a part of the saponification is effected by treatment with an aqueous liquid medium which contains a water-soluble nitrogenous organic base in which each carbon atom that is directly attached to a nitrogen atom is directly attached to three other atoms apart from said nitrogen atom, and the desired saponification is completed by a subsequent treatment with a mineral saponifying agent.

4. Process for saponifying filaments, threads, fibres, ribbons, films and like materials having a basis of organic ester of cellulose, wherein a part of the saponification is effected by treatment with a lower aliphatic amine, and the desired saponification is completed by a subsequent treatment with a mineral saponifying agent.

35 5. Process for saponifying filaments, threads, fibres, ribbons, films or like materials having a basis of cellulose acetate, wherein the materials are first treated with an aqueous solution of methylamine until the acetyl content corresponds to not more than one acetyl group per  $C_6H_{10}O_5$  unit, and the desired saponification is then completed by a subsequent treatment of the materials with an aqueous solution of a caustic alkali.

45 6. Process for saponifying filaments, threads, fibres, ribbons, films or like materials having a basis of cellulose acetate, wherein the materials are first treated with an aqueous solution of ethylene diamine until the acetyl content corresponds to not more than one acetyl group per  $C_6H_{10}O_5$  unit, and the desired saponification is

then completed by a subsequent treatment of the materials with an aqueous solution of a caustic alkali.

7. Process for saponifying filaments, threads, fibres, ribbons, films and like materials having a basis of cellulose acetate, wherein the materials are treated, first with a 15 to 30% aqueous solution of methylamine containing 0.05 to 0.5% copper at a temperature between 30 and 60° C. until the acetyl content of the ester corresponds to not more than one acetyl group per  $C_6H_{10}O_5$  unit, and the materials are then immediately treated with an aqueous solution containing 1 to 3% caustic soda at a temperature above 90° C. until the acetyl content is substantially completely removed.

15 8. Process for saponifying filaments, threads, fibres, ribbons, films and like materials having a basis of organic ester of cellulose, wherein the saponification is partly effected by treating the materials with a lower aliphatic amine until the cellulose ester contains not more than  $1\frac{1}{2}$  acetyl groups per  $C_6H_{10}O_5$  unit, and the desired saponification is completed by a subsequent treatment with a mineral saponifying agent.

20 9. Process for saponifying filaments, threads, fibres, ribbons, films and like materials having a basis of cellulose acetate, wherein a part of the saponification is effected by treatment with a lower aliphatic amine, and the desired saponification is completed by a subsequent treatment with a mineral saponifying agent.

25 10. Process for saponifying filaments, threads, fibres, ribbons, films and like materials having a basis of cellulose acetate, wherein a part of the saponification is effected by treatment with methylamine, and the desired saponification is completed by a subsequent treatment with a mineral saponifying agent.

30 11. Process for saponifying filaments, threads, fibres, ribbons, films and like materials having a basis of cellulose acetate, wherein a part of the saponification is effected by treatment with ethylene diamine, and the desired saponification is completed by a subsequent treatment with a mineral saponifying agent.

35 ROBERT WIGHTON MONCRIEFF.  
FRANK BRENTNALL HILL.

CERTIFICATE OF CORRECTION.

Patent No. 2,092,010.

September 7, 1937.

ROBERT WIGHTON MONCRIEFF, ET AL.

It is hereby certified that error appears in the printed specification of the above numbered patent requiring correction as follows: Page 1, second column, line 41, for the words and syllable "or higher fatty acid esters, for ex—" read of higher fatty acids, for example; and that the said Letters Patent should be read with this correction therein that the same may conform to the record of the case in the Patent Office.

Signed and sealed this 2nd day of November, A. D. 1937.

(Seal)

Henry Van Arsdale,  
Acting Commissioner of Patents.